

## UNITED STATES PATENT OFFICE

PAUL GAMICHON, OF PARIS, FRANCE

PROCESS FOR CONVERTING INTO SOLUBLE SALTS LEAD AND OTHER METALS CONTAINED  
IN LEAD BEARING ORES

No Drawing. Application filed June 12, 1931, Serial No. 543,819, and in France June 17, 1930.

The various known processes for roasting lead-bearing sulphide ores with a view to their subsequent treatment by dissolution and wet means may be restricted to two:

5 (1) Sulphating roasting. In this case, the conversion of the sulphide ore is somewhat slow and difficult to carry out. It is, furthermore, always very incomplete.

10 (2) Chlorinating roasting. In this case, to be complete, the reaction requires a considerable excess of alkaline or earth-alkaline chloride, the cost of which renders its use prohibitive. It requires a somewhat high temperature (dark red at least) whereby considerable volatilization of the heavy metal chlorides is caused and especially those of lead.

15 Furthermore, neither of these roasting processes can be used successfully to bring to the condition of soluble salts the whole of the metals contained in the ores. If roasting is continued too long or if too high a temperature is applied, oxides are formed, and sometimes even the metal itself is reached and in 20 all cases heavy losses are incurred due to the volatilization of the sulphate or chloride.

25 The process pursuant to this invention consists essentially in combining a chlorinating and sulphating roasting with a subsequent 30 treatment of the roasted material by means of a strong acid and thereafter by means of a brine.

35 The first step consists in roasting the ore in the presence of both a small quantity of sulphate of lime and of a quantity of alkaline chloride or of earth-alkaline chloride which is very much less than the theoretical amount needed to chlorinate the whole of the lead. The ore is thereby very quickly rid of 40 sulphur while furnishing a mixture of lead chloride and sulphate.

45 It would appear that, in point of fact, the alkaline or earth-alkaline chloride used acts only as a catalytic agent in the desulphurizing of the lead.

50 The process may be carried out in an ordinary roasting oven (Wedge or any other) with an air inlet and it requires a moderate temperature only.

50 The reaction so obtained is much faster

and more complete than is the case in roasting which is solely sulphating, notwithstanding the small proportion of added chloride. By this means, furthermore, all formation of oxide (PbO) is practically avoided, which is 55 impossible in the case of sulphating roasting.

The roasted material, containing especially sulphates and chlorides which have been formed, is then treated by means of a small quantity of strong acid, corresponding only 60 to the quantity of sulphide which has not been converted by roasting.

Should the acid used be sulphuric acid, the traces of galena or of sulphides which have not been converted, together with the traces 65 of oxides, are converted into sulphates.

The sulphates of soluble metals (Zn, Cu, etc.) are easily separated by washing and their solutions may be treated subsequently by one of the usual methods. 70

In place of sulphuric acid, hydrochloric acid and other strong acids having the same properties may be used, with corresponding differences in results with respect to the salts obtained. 75

If the remainder of the roasted ore be thereafter washed hot with brine, the whole of the lead and silver is recovered as soluble chlorides, which is impossible with any of the known roasting processes. 80

The chloride of lead thus obtained may be crystallized or be used for the preparation of metallic lead or compounds thereof by any known method.

The process is exemplified by the following 85 illustration which does not restrict the scope of the invention:

1000 kg of ore is crushed, which contains as sulphides 300 kg lead and 150 kg zinc, as well as 400 grams silver and 1500 grams copper, so that the whole is adapted to pass through a sieve of approximately 20 mesh. 90

The ore thus crushed is thereupon mixed with 80 kg at least of chloride of sodium and 20 kg  $\text{CaSO}_4$  and the whole mass is roasted in 95 an oxidizing atmosphere, the temperature being gradually raised to  $460^\circ$ - $490^\circ$  C.

As soon as this temperature is reached, reaction takes place almost immediately.

The roasted ore is thereupon washed with 100

500 litres of water containing 15 litres  $\text{SO}_4\text{H}_2$  at 53-55 Bé. This washing completes the conversion of the insoluble salts into soluble salts and the whole of the zinc, copper and other soluble metals may be eliminated by lixiviation and filtration.

The remaining roasted ore which contains lead, is then lixiviated with 4 cubic metres of a brine containing at least 250 grammes of 10  $\text{NaCl}$  per litre and a total quantity of 6 litres of commercial  $\text{HCl}$  (22 Bé.). The solution is kept at a temperature of 85-100° C. and in half an hour, the whole of the lead, silver and other metals will be found to have passed 15 into solution.

The iron, alumina, silica and manganese are precipitated in the hot liquor, before filtration, by any known means.

The liquor is then filtered while hot, crystallization is obtained and some 225 to 230 kg lead is thus secured as crystallized chloride.

The silver, for example, may be precipitated in mother-lyes containing spongy lead 25 obtained in any known manner. The mother-lyes containing lead may be used afresh, to dissolve the lead contained in the roasted ore of another cycle of operations.

I claim:

30 1. Process for converting into soluble salts metals contained in lead bearing sulphide ores, which consists in roasting said ores at a moderate temperature in the presence of a small quantity of sulphate of lime and of alkaline or earth-alkaline chlorid, then in treating the roasted material successively with a strong acid having the property of converting into soluble salts the sulphides or traces of oxides left unconverted after roasting, lixiviating the mass to separate the salts of soluble metals, such as those of zinc or copper, and treating with a brine to bring into solution the lead, the silver and the metals associated therewith.

40 2. Process for converting into soluble salts metals contained in lead bearing sulphide ores, which consists in roasting said ores at a moderate temperature in the presence of a small quantity of sulphate of lime and of alkaline or earth-alkaline chlorid, then in treating the roasted material with sulphuric acid to convert into sulphates the sulphides or traces of oxides left unconverted after roasting, and in lixiviating the mass to separate 50 the salts of soluble metals, such as those of zinc or copper, and in treating with a brine to bring into solution the lead, the silver and the metals associated therewith.

3. Process for converting into soluble salts 60 metals contained in lead bearing sulphide ores, which consists in roasting said ores at a moderate temperature in the presence of a small quantity of sulphate of lime and of alkaline or earth-alkaline chlorid, then in 65 treating the roasted material with hydro-

chloric acid to convert into chlorides the sulphides or traces of oxides left unconverted after roasting, and in lixiviating the mass to separate the salts of soluble metals, such as those of zinc or copper, and in treating with 70 a brine to bring into solution the lead, the silver and the metals associated therewith.

4. Process for converting into soluble salts metals contained in lead bearing sulphide ores, which consists in roasting said ores at 75 a moderate temperature in the presence of a small quantity of sulphate of lime and of alkaline or earth-alkaline chlorid used in much smaller quantity than the theoretic amount required to chlorinate the whole of the lead 80 of the ore, then in treating the roasted material successively by a strong acid having the property of converting into soluble salts the sulphides or traces of oxides left unconverted after roasting, and then with a brine.

5. Process for converting into soluble salts metals contained in lead bearing sulphide ores, which consists in roasting said ores at a moderate temperature in the presence of a small quantity of sulphate of lime and of alkaline or earth-alkaline chlorid, in treating 90 the roasted material by sulphuric acid so as to convert into sulphates the sulphides or traces of oxides left unconverted after roasting, and in lixiviating the mass to separate the salts 95 of soluble metals, such as those of zinc or copper, and in treating with a brine to bring into solution the lead, the silver and the metals associated therewith, and finally in filtering the hot liquor obtained after precipitation of 100 metals other than lead and silver and in cooling said liquor for the crystallization of the chloride of lead.

In testimony whereof I have signed this specification.

PAUL GAMICHON.

105

110

115

120

125

130